

Patented July 28, 1925.

1,547,927

# UNITED STATES PATENT OFFICE.

ALAN KISSOCK, OF LOS ANGELES, CALIFORNIA, ASSIGNOR TO CARL M. LOEB, OF NEW YORK, N. Y.

## PROCESS OF MAKING ALLOY STEEL.

No Drawing.

Application filed May 21, 1924. Serial No. 714,769.

*To all whom it may concern:*

Be it known that I, ALAN KISSOCK, a citizen of the United States, residing at Los Angeles, in the county of Los Angeles and State of California, have made a certain new and useful Improvement in Processes of Making Alloy Steel, of which the following is a specification.

The invention relates to a process of making alloy steel, and the objects and advantages thereof will be set forth in part hereinafter and in part will be obvious herefrom or may be learned by practice with the invention.

15 The invention consists in the novel steps and processes herein described.

In my copending application Ser. No. 703,533 I have described and claimed a process whereby I have effected a desired 20 definite chemical combination between certain of the naturally occurring constituents of many molybdenum ores, thereby producing molybdates of the general formula,  $ROMoO_3$ ,  $R_2O_3MoO_3$ , and more especially 25 an iron molybdate or molybdates. Dependent upon the type of steel into which it may be introduced, such an iron molybdate may be a chemically precipitated powder product, containing substantially only the elements 30 iron, molybdenum and oxygen; or it may be a sintered product, directly from the roasting operation, and in addition to iron, molybdenum and oxygen may contain certain of the foreign constituents of the ore.

35 The present invention provides a process of alloying steel, and more especially alloying steel with such a chemically combined molybdenum, without requiring any preliminary metallurgical operation to prepare 40 the molybdenum for the alloying process.

An example of the usual preliminary metallurgical operations referred to is the reduction of the molybdenum ore to what is known as the ferro state, that is, making a 45 mixture of molybdenum and iron, both being usually included in relatively large proportions, thereby to prepare the molybdenum for the process of alloying in the steel-making furnace, and during the steel-making 50 operation. Such a mixture of the two metals is known as ferro-molybdenum.

The invention is further directed to providing a process whereby steel may be alloyed with molybdenum directly from a 55 molybdate without presenting to the steel

furnace or its contents an irreducible component or material, which is frequently perniciously chemically active, and thereby also avoiding the creation of a slag.

The invention is further directed to providing a process especially advantageous for the acid open-hearth furnace, for crucible steel making, and for other processes wherein in the making of slag, or the releasing from the alloying material of an active chemical 65 component or constituent, which might deterioriously affect the apparatus or the product, is undesirable or detrimental.

By my process I introduce into the steel-making furnace a molybdenum chemical compound, all, or all the important, ingredients or elements of which are capable of combining with the steel then in the furnace.

In practicing my process ferric molybdate, or other iron molybdate, is introduced 75 into the steel-making furnace at some time during the steel-making operation. Under usual steel making conditions, the complete reduction of the molybdate or molybdenum chemical compound, and its incorporation 80 into the steel as an alloy, requires several hours, and it is preferable to add or insert the molybdate in the early stages of the heat of steel.

Both constituents of the compound are 85 dissociated from their chemical combination, and are capable of being reduced to their respective metallic states, namely, iron and molybdenum (by the carbon or some other element or materials ordinarily present in 90 the steel or steel furnace). These component elements may, and preferably do, practically completely unite with and are entirely absorbed by the steel, and there is no formation at least to any material degree of 95 any interfering slag or other objectionable or deleterious substance.

Thereby the serious disadvantage of alloying with the steel a compound or substance one component of which is irreducible under steel furnace conditions is avoided. For instance, where the compound used in the alloying process contains a basic element which is not reduced to the metallic state under steel furnace conditions, two distinct steps or reactions are involved, namely reduction and combination. The molybdenum component of the compound must first be reduced to the metallic state, and the basic component is then free and must combine 100 105 110

with some acid constituent present in the furnace. In the case of the acid open-hearth steel process, this acid constituent with which the non-reducible basic alkaline component must unite to form a slag is often the lining of the furnace itself, which is thereby corroded and requires replacement. The crucible steel process is essentially a melting, and not a refining process and the production of any slag must be avoided.

In distinction to this, iron molybdate, both components of which are not only capable of reduction under a steel furnace conditions, but both elements of which may also be absorbed or alloyed with the steel itself, offers a molybdenum compound entirely suitable for all steel making processes, and is entirely free from the disadvantages enumerated. The costly preliminary or outside reduction of a molybdenum ore to what is commonly known as a ferro alloy, and the undesirable chemical action of other molybdenum compounds, is avoided.

It will be understood that there may be

departures from the details of the practice of my invention, as herein described, without departing from the principles thereof and without sacrificing its chief advantages.

What I claim is:—

1. The process of making molybdenum steel comprising adding iron molybdate directly to the steel furnace during the process of making the steel, whereby the iron molybdate is reduced by the constituents of the steel bath, no other reducing agent being added to effect such reduction.

2. The process of making molybdenum steel comprising adding a charge consisting of substantially pure iron molybdate, with no other reacting material therein, directly to the steel furnace during the process of making the steel whereby the iron molybdate is reduced by the steel itself without the use of any other reducing agent.

In testimony whereof, I have signed my name to this specification.

ALAN KISSOCK.